

July 26, 1955

W. J. BURGON

2,714,081

PROCESS OF FORMING FIBROUS SHEETS

Filed March 17, 1950



INVENTOR.  
William J. Burgon  
BY  
*Buckhorn and Cheatham*  
Attorneys

1

2,714,081

## PROCESS OF FORMING FIBROUS SHEETS

William J. Burgon, New Westminster, British Columbia, Canada, assignor of fifty-one per cent to William H. Rambo, Portland, Oreg.

Application March 17, 1950, Serial No. 150,204

3 Claims. (Cl. 154—101)

The present invention comprises a method and apparatus for forming fibrous sheets such as fiberboards, fibrous core stock, fiber insulating pads and similar items of a self-sustaining nature, being particularly concerned with fiber articles of a planular form and of a density of about .7 or less. Material formed in the apparatus and by the method of my present invention may later be subjected to heat and pressure to form hard fiberboard of a density in the range of 1.0 by any of the known processes and utilizing any known apparatus, and I do not intend to exclude from the purposes of my invention the thought of forming articles of such hardness but am limiting the disclosure and claims of this application to the inventive features involved in the formation of a sheet of fibers of an intermediate or low density utilizable either as the end product or as an intermediate product in the formation of articles of high density.

The invention relates to the formation of medium or low density products by the use of lignocellulosic materials reduced to a finely divided or fibrous condition and rendered plastic, immediately upon rendering the fibers plastic rather than at a later stage as is the case with all processes with which I am at present acquainted. The art of making fibrous sheet materials as presently practiced comprises the reduction of lignocellulosic materials to a fibrous condition and the rendering of the same to a plastic state in the presence of hot water or steam, by means of equipment and processes such as disclosed, for example, in the patents to Asplund 2,008,892, July 23, 1935, and 2,145,851, February 7, 1939, or in the patents to Mason 1,578,609, March 30, 1926, and 1,586,159, May 25, 1926, or in the patents to Mason 1,663,503, 1,663,504, 1,663,505 and 1,663,506, all of March 20, 1928. In all of these prior art processes the hot, plasticized fibers are subjected to further treatment in which they lose their plasticity and become inert, hardened, or relatively cool fibers incapable of cohering to each other until they are again brought back to a condition of plasticity by the further application of heat. All such processes involve the mixing of the fibers with sufficient water to permit pumping the mixture from place to place; and finally the dense pulp is mixed with water at a temperature insufficient to plasticize the fibers and in such large quantity as to form a slurry having the flowing characteristics of water. The slurry is agitated to maintain the fibers in suspension while the water is brought into contact with a screen through which the water is drained while a mat of cold fibers is deposited upon the screen. The so-called "white water" drained from the fibers contains recoverable valuable substances such as fibers themselves or chemicals such as fillers, sizes, resins and the like which have been mixed with the pulp or the slurry at some stage in the process preceding the screening operation, hence the white water has to be recaptured and the valuable components recovered by some means. The so formed mat of fibers usually contains a large quantity of free water which is removed from the mat so as to

2

economize on the heat required to reheat the fibers to a condition of plasticity in a subsequent heating and pressing operation where the mat is reduced to a self-sustaining sheet of the desired characteristics, the amount of pressure, the amount of heat applied and the duration of application of either or both being regulated to determine the density and other characteristics of the resulting sheet. All such steps subsequent to the initial formation of the plastic fibers require far greater expenditure of energy, far greater equipment and far greater man-hours of labor than that required initially to reduce lignocellulosic fibers to a disintegrated, plastic condition. It is the principal object of the present invention to eliminate all such intermediate steps and apparatus and to form self-sustaining sheet material directly from the plastic fibers created in such equipment as an Asplund defibrator or other equipment for producing plastic fibers.

The foregoing and other objects and advantages of the present invention will be more readily ascertained from inspection of the following specification taken in connection with the accompanying drawing wherein like numerals refer to like parts throughout, while the features of novelty will be more distinctly pointed out in the appended claims.

In the drawing,

Fig. 1 discloses one type of equipment which may be utilized to receive the output of a plastic fiber producing mechanism and form self-sustaining fiber sheets therefrom; and

Fig. 2 illustrates a second form which may be utilized.

The drawing schematically discloses two types of equipment which may be utilized in carrying out my process, the two types having general characteristics in common and being merely exemplary of many different forms which the apparatus may assume without departing from my invention.

Referring to Fig. 1, there is disclosed at 10 a box exemplifying equipment for forming plastic lignocellulosic fibers, which equipment may be as disclosed in the above-identified Mason patents, but which is preferably of the type disclosed in the above-identified Asplund patents because the Asplund equipment produces a more nearly continuous flow of hot, plasticized fibers. In the Asplund equipment wood chips or the like are continuously fed to internal mechanism for beating, rubbing or agitating the chips after they have been subjected to steam at such temperatures and pressures as substantially to plasticize the fibers in a relatively short time, the mechanical agitation or beating thereupon readily disintegrating the chips or the like and separating the individual fibers in an envelopment of steam. The apparatus may be of the continuous flow type in which pressure is maintained by an outlet restriction, or may be of the substantially continuous flow type in which continuity of flow is established while maintaining high pressures within the equipment by intermittently opening and closing a valve at the output end of the equipment, each opening of the valve resulting in the discharge of a plug of plasticized fibers under steam pressure such that the steam may be utilized to convey the fibers to other equipment. The box 10 may exemplify any other type of equipment from which a relatively continuous flow of fibers in an environment or envelopment of steam is emitted into a discharge pipe 11. The box 10 may, for example, represent a plasticizer which receives the output of other defibrating equipment such as mechanical grinders or plasticizers as disclosed in the Mason patent, thereby providing means for producing relatively continuous and uniform flow of hot, plasticized fibers from intermittently or continuously discharging equipment. The box 10 may represent an Asplund machine receiving

the output of some other type of disintegrating equipment such as wood grinders or the like. My invention therefore comprises a closed vessel 10 in which fibers are rendered plastic by subjecting them to steam at such temperatures and pressures and for such lengths of time as may be required by the characteristics of the fibers. As is well known in the art and thoroughly explained in the above-mentioned Asplund patent 2,008,892, the steam may be at or near the boiling point of water but is preferably at a higher temperature achieved by holding the pressure at greater than atmospheric. Best results are obtained when the temperature is maintained between 250° F. and 360° F. The temperature should not be materially above 400° F. as such elevated temperatures do not materially facilitate the disintegration or plasticizing of the fibers and charring or discoloration of the fibers usually takes place at elevated temperatures of the order of 450° F. to 500° F. In an Asplund machine wood fibers subjected to temperatures between 300° F. and 340° F. for some twenty to forty seconds, depending upon the original moisture content and temperature of the wood, will be reduced to substantially individual fibers or bundles of fibers of such size as to be suitable for the formation of boardlike materials in the equipment and will be ejected therefrom in a plastic state in an environment of steam under pressure.

Instead of conducting the steam-borne fibers to a cyclone or other equipment in which the fibers are separated from the steam and dropped into storage or treating vats where it is allowed to cool and is mixed with diluting water, my invention contemplates the provision of a relatively thin, wide discharge spout 12 directly connected to a short outlet pipe 11 from the equipment 10, the orifice 13 of the flaring outlet being located in the angle of convergence between a supported, traveling screen 14 and an opposed driven, heated roll 15. In the embodiment disclosed in Fig. 1 the screen 14 is supported upon a perforated cylinder 16 of relatively large diameter, and a spaced stretcher roll 17 of any suitable diameter. The roll 15 may have any desired diameter provided that the surface speed thereof is the same as the surface speed of the screen 14. The distance between the rolls 15 and 16 is such that a layer of fibers in hot, plastic condition enveloped in steam will be deposited upon the screen between the two rolls. The speed of movement of the screen and the opposed roll 15 should be such as to cause a plug of fibers continuously to form at the orifice 13 or in spout 12 behind the orifice 13, thus holding the steam pressure in the outlet and creating a uniform layer by eliminating the pulsations of discharge from the equipment 10. The plug will not be of such density as to prevent the continuous escape of steam therefrom so that the fibers are compacted and interlaced with each other in the longitudinal direction of the layer being deposited upon the traveling screen.

The screen 14 may be of any suitable type developed in the pulp and paper industries and may comprise a woven wire screen or other foraminous member such as a perforated, flexible sheet. The drum 16 preferably has perforations of larger diameter but still of relatively small size and closely spaced throughout so that upon the application of suction to the interior of the drum the steam will be uniformly withdrawn from the hot mat.

The mat while sustained upon the drum is successively compressed and released by the application of rolling pressure thereto through the medium of a series of heated pressing rolls 18, 19 and 20 which may be disposed at successively decreasing distances from the surface of the wire or may be uniformly spaced therefrom, depending upon the density and other characteristics of the sheet to be formed. While being alternately compressed and released from pressure the mat is subjected to suction by the application of suction to the interior of the drum so that the steam is rapidly withdrawn from the fibers after the initial compression applied by roll 15, and heated air is

drawn through the fibers to maintain them in somewhat plasticized condition while the subsequent pressing operations are taking place. It may be desirable in some cases not to draw air between the rolls 18, 19 and 20, in order that the fibers will remain plasticized for a longer time, this condition being maintained by the heated rolls.

Preferably the space between rolls 15 and 18 is sealed from the outer atmosphere by an intermediate sealing roll 21, the rolls 15, 21 and 18 thereby providing a chamber 10 22 into which steam may be injected through the medium of perforated pipes indicated at 23 and 24. The plasticity of the fiber may thus be more gradually reduced, lending greater effect to the compressing action of the second roll 18. A further function may be provided in that one of 15 the pipes, such as the pipe 23 may be utilized for the injection of steam and the other pipe utilized for the application of some foreign chemical such as an insect poison, antifungus chemical, sizing material, resin, or coloring matter. It is to be appreciated that no binder need be 20 added, but that resin binders or the like may be added for special purposes. Preferably the pipe 23 would be utilized for introducing such foreign substances, and the pipe 24 utilized for the introduction of steam serving to drive the 25 chemical or foreign substance into more intimate contact with the fibers and distribute the same more evenly through the mat.

The drum 16 is preferably of the type driven through end bells or the like so that the interior may be subdivided into stationary compartments to which suction may 30 be individually applied, the partitions being such as disclosed at 25, 26 and 27 providing a pair of interior suction chambers 28 and 29 to which suction may be applied individually through pipes 30 and 31. The partition 25 may be arranged to permit drainage of condensed steam or 35 other liquid material to a low point so that water will not remain in the chamber 28 and so that any chemical which may be carried through the mat may be salvaged. A further function is achieved in this fashion in that the steam which is substantially entirely withdrawn from the mat in 40 the space between the points of contact of rolls 18 and 15 may be utilized initially to heat the lignocellulosic material, thus further reducing fuel consumption.

The drum 16 should be of such relatively large diameter that the mat upon leaving the surface of the drum and 45 following the stretch of wire between the drum 16 and stretcher roll 17 will not crack to any appreciable extent along its lower or wire surface. However, there might be a multiplicity of fine checks or cracks in the lower surface of the sheet, and for this purpose a succeeding 50 pair of pressure rolls 32 and 33 further compact the mat as it travels toward the stretcher roll 17, this action taking place while the fibers are still in somewhat plastic condition and before they become permanently set. Further pressure is preferably provided by a roll 34 opposing the 55 stretcher roll 17. At this point the mat would be self-sustaining and in condition to travel straight ahead while the screen separates therefrom, around the stretcher roll 17, and would be carried from the forming equipment by 60 suitable means such as the carrier rolls 35. The sheet may be conducted by the carrier rolls into any desired finishing equipment.

It is to be appreciated that at this point a self-sustaining, continuous sheet of medium or low density is formed. This sheet is cut into smaller sheets which may be conducted to a storage space and may be utilized in their 65 existing shape as insulating material, pads, acoustic surfacing or core stock. However, if denser or smoother boards are desired, they may be removed from the storage space, or conducted directly from the forming equipment, and placed in or passed through equipment adapted to 70 apply heat and pressure to create hardboard or other sheet material of greater density or otherwise finish the material, as is well known in the art.

In order to demonstrate that the present invention is 75 not limited to a particular type of equipment; and in order

to illustrate a type of equipment in which it will be certain that no checking or cracking of the wire surface of the sheet will occur, I have illustrated a second form in Fig. 2. In this form the fibers are plasticized in equipment indicated at 40 and conducted through pipe 41 and a flaring outlet 42 to an orifice 43 in the angle of convergence between the upper flight of a traveling screen 44, entrained about end rolls 45 and 46, and a first heated pressure roll 47. The upper flight of the wire is supported upon a grid or perforated plate 48 beneath which is positioned suction means such as a first suction box 49 and a second suction box 50. The suction box 49 is preferably coextensive with the space between the point of contact of the first presser roll 47 and a second presser roll 51. The space between rolls 47 and 51 is formed into a chamber 52 by a sealing roll 53, and a pair of pipes 54 and 55 may introduce steam and/or other materials into the chamber so as to be sucked through the mat into the box 49 and salvaged through the suction pipe 56. A plurality of other heated presser rolls 57, 58 and 59 successively apply rolling pressure to the mat while on the screen, the rolls being spaced to permit the passage of air therebetween upon the application of suction to the box 50 through the pipe 60. By the time the mat passes from the opposed rolls 46 and 59 a self-sustaining sheet of medium or low density will be formed and may be transported away from the forming apparatus by carrier rolls 61. In this instance I have illustrated further treating equipment such as a pair of opposed pressing rolls 62 and 63 which are preferably heated and which further compact the sheet and exemplify other equipment which may be utilized to produce a finished product of high density.

It is to be appreciated that the apparatus herein disclosed is schematically illustrated. For example, no details are given of equipment which may be utilized to synchronize the feeding movement of the screen with the rate of production of the fibers. For example, means may be supplied at or near the orifice of the conduit conducting the fibers to the screen for sensing the volume of fibers being ejected or for sensing the thickness of the mat at the point of formation and controlling the speed of the screen and rolls accordingly, thereby continuously to assure uniformity of the mat being formed. Under normal conditions such would not be necessary since the equipment for forming the plasticized fiber would be of such capacity as to be capable of producing plasticized fibers at a rate to insure the formation of a uniform layer at the desired constant rate of movement of the screen, the initial compressing roll ironing out irregularities in a lateral direction and holding back a plug within the flaring tube. Sensing equipment may be placed in, or arranged in conjunction with, the flaring outlet tube to regulate the speed of operation of the plasticizing equipment so as to insure the formation of a uniform mat. It is to be appreciated that the present invention may be utilized in the formation of mats from fibers created in any suitable manner provided that they are rendered plastic and fed to the screen in a hot, plastic condition in a gaseous environment rather than in liquid suspension. By the term "steam" I mean to imply the usual definition thereof as water in a gaseous state, with or without the addition of other impurities such as would be present in the lignocellulosic materials or which may have been added in the treatment thereof.

Having illustrated and described preferred embodiments of my invention, it should be apparent to those skilled in the art that the invention permits of modification in arrangement and detail. I claim as my invention all such modifications as come within the true spirit and scope of the appended claims.

I claim:

1. The process of making fiber boards comprising subjecting lignocellulosic fibers to steam in a high pressure zone until the fibers are plasticized, permitting the continuous escape of steam to a zone of steam at lower pressure and utilizing the steam to entrain fibers in hot, plasticized condition, resisting movement of the entrained fibers at the point of release from the zone of high pressure so as to build up a wall of interlaced fibers between the two zones of pressure, continuously and mechanically withdrawing the built-up wall of fibers through the zone of lower pressure steam so as to form a continuous mat of plasticized fibers interlaced in the longitudinal direction of the mat, and compressing the mat into a self-sustaining sheet while moving the same away from association with steam.
2. The process of making fiber boards or similar fibrous sheets comprising subjecting lignocellulosic fibers to steam under pressure in a confined space until the fibers are plasticized, continuously releasing the plasticized fibers from the confined space in a relatively thin, wide stream under pressure of steam escaping from the confined space, mechanically moving the fibers away from the point of release from the confined space at a rate such that pressure is maintained in the confined space and a continuous mat of fibers is formed, and subjecting the moving mat to transverse compression until the fibers lose plasticity.
3. The process of making fiber boards or similar fibrous sheets comprising subjecting lignocellulosic fibers to steam under pressure in a confined space until the fibers are plasticized, continuously releasing the plasticized fibers from the confined space in a relatively thin, wide stream under pressure of steam escaping from the confined space, mechanically moving the fibers away from the point of release from the confined space at a rate such that pressure is maintained in the confined space and a continuous mat of fibers is formed, and transversely compressing the moving mat while subjecting the mat to suction applied to at least one surface thereof to hasten the withdrawal of steam therefrom.

#### References Cited in the file of this patent

#### UNITED STATES PATENTS

|           |                |                |
|-----------|----------------|----------------|
| 1,927,361 | Edge           | Sept. 19, 1933 |
| 2,080,078 | Mason          | May 11, 1937   |
| 2,145,851 | Asplund        | Feb. 7, 1939   |
| 2,189,840 | Simison et al. | Feb. 13, 1940  |
| 2,329,799 | Thorsen        | Sept. 21, 1943 |
| 2,345,647 | Witham         | Apr. 4, 1944   |
| 2,369,653 | Berry          | Feb. 20, 1945  |
| 2,427,495 | Deuchler       | Sept. 16, 1947 |
| 2,480,851 | Goss           | Sept. 6, 1949  |
| 2,543,101 | Francis        | Feb. 27, 1951  |
| 2,544,019 | Heritage       | Mar. 6, 1951   |
| 2,553,412 | Heritage       | May 15, 1951   |
| 2,577,205 | Meyer et al.   | Dec. 4, 1951   |